# EUROPEAN PATENT SPECIFICATION

(11) **EP 0 089 113 B1**
(45) Date of publication and mention of the grant of the patent: **13.05.1987**
(21) Application number: 83300640.6
(22) Date of filing: 09.02.1983
(51) Int. Cl.: D01F 8/06, D01F 1/10

(54) **Fire retardant composite fibres and process for producing them**
Flammhemmende zusammengesetzte Fasern und Verfahren zur Herstellung derselben
Fibres composites retardant la flamme et procédé pour leur fabrication

(30) Priority: 12.03.1982 JP 39167/82
(43) Date of publication of application: 21.09.1983
(73) Proprietor: Chisso Corporation, Osaka-shi Osaka-fu (JP)
(72) Inventor: Goi, Shigeru, Moriyamashi Shigaken (JP); Sugihara, Taizo, Moriyamashi Shigaken (JP)
(74) Representative: Ruffles, Graham Keith

## Description

This invention relates to fire retardant composite fibres and a process for producing them. More particularly it relates to polyolefin composite fibres comprising two kinds of polyolefin polymers having different melting points and having the same or different fire retardants in the two components.

Polyolefin composite fibres have superior heat adhesive properties and also physical and chemical properties and further are light weight and cheap; hence they have been used as a fibre material for non-woven fabrics in various applications fields. For example, they are suitable as a material for thin products such as fabric bases, hygienic materials, napkins, paper diapers, and for thick products such as quilting goods, various felts, filters, fibre-shaped products, materials for public works, etc. In general, fire retardant properties have been used indoors for fibre materials. As a process for making polyolefin fibres fire retardant, there is first a process of adding a fire retardant to raw material polymers, followed by spinning. Also JP-A-5658009 discloses the addition of 0.5-5% by weight of fire retardant, based upon the lower melting component, to only the lower melting component of a polyolefin composite fibre and stretching the spun fibers to 4-8 times their original weight. As a result, it is said that the fire retardancy is superior to the case where the same amount of fire retardant is added to each component. However, addition of fire retardants in a large amount raises various problems of reduction in productivity and product quality, etc., such as obstacles at the time of spinning and stretching e.g. fibre breakage, reduction in strength, rough fibre surface, reduction in heat adhesive properties, etc. These problems are notable in the case of thin fibres of 6 d/F (6.7 dtex/F) or less; and particularly in the case of composite fibres, they notably appear on the side of lower melting component having a lower viscosity. A method of providing the required degree of fire retardancy, particularly to polyesters and polyamides, without bringing about the difficulties discussed above is described in US-A-3658634. US-A-3658634 discloses a sheath and core type conjugate fibre obtained by providing a core composed of polymer prepared by blending a specific halogen substituted aromatic compound and phosphorus compound in predetermined amounts and by wrapping the core component with a sheath component. Further, beside the above-mentioned process, processes of coating fibres with a fire retardant or blending fire retardant fibres have been known, but in the case of these processes, since shaped fibres are treated by post-processing, the steps are complicated, the quality fluctuation is large and the cost is high; hence these processes are not practical.

The present inventors have made various studies on such problems and found that when the higher melting and lower melting components of composite polyolefin fibres respectively contain a fire retardant having a decomposition temperature higher than the melting points of the respective components by 100°C or more and also having a particle size of 62 um or less, it is possible to produce superior fire retardant and heat adhesive composite fibres of a small denier having a relatively large amount of the fire retardant blended also with the lower melting component, with a good spinnability.

One aspect of the present invention resides in:
fire retardant composite fibres comprising a fibre-formable polyolefin polymer as a higher melting component and a polyolefin polymer having a melting point lower than that of the higher melting component by 10°C or more, as a lower melting component, and having a fire retardant contained in the respective components,
which composite fibres are characterized in that a fire retardant having a decomposition temperature higher than the melting points of the respective components by 100°C or more and also having a particle size of 62 µm or less, is contained in the respective components in an amount of 3 to 15% by weight, and the total of the respective amounts of the fire retardant contained in the whole of the composite fibres is 5 to 10% by weight.

Another aspect of the present invention resides in:
a process for producing fire retardant composite fibres by using a fibre-formable polyolefin polymer having a melting point lower than that of the higher melting component by 10°C or more, as a lower melting component, blending a fire retardant with the respective components and subjecting the resulting components to melt-composite-spinning followed by stretching,
which process is characterized by blending a fire retardant having a decomposition temperature higher than the melting points of the respective components by 100°C or more and also having a particle size of 62 pm or less, with the respective components, so as to give an amount of the fire retardant of 3 to 15% by weight, and also so as to give the total of the respective amounts of the fire retardant contained in the whole of the composite fibres, of 5 to 10% by weight; melting the resulting components at a temperature lower than the respective decomposition temperatures of the fire retardant contained in the respective components to subject them to composite spinning.

In general, in the case of composite fibres, it is possible to impart various specific features to their crimpability and adhesive properties, depending on the combination manner of composite components, and it is also possible to use the fibres in application fields corresponding thereto. Composite fibres of the present invention also have various application fields, and it is particularly preferable for them to be a side by side or a sheath and core type, so that the lower melting component can have a percentage fibre-cross-sectional circumference of 50% or higher, thereby to provide the composite fibres provided with heat adhesive properties by way of the lower melting component. In this case, the composite ratio (higher melting component: lower melting component) is preferably in the range of 5:5 to 3:7 in view of the thickness of the lower melting component in the fibre section.

The higher melting component is preferably polypropylene or copolymers composed mainly of propylene having a fibre formability. The lower melting component is preferably polyethylene, ethylene-vinyl acetate copolymers, abbreviated to EVA, having a vinyl acetate content of, e.g. 1 to 10% by weight, their saponified products, blends of polyethylene with EVA or saponified EVA.

The respective contents of the fire retardant in the high melting component and the lower melting component of the composite fibres are suitably in the range of 3 to 15% by weight, and the total content of the fire retardant in the whole of the composite fibres is suitably in the range of 5 to 10% by weight. If the contents of the fire retardant are lower than the above ranges, the fire retardant effectiveness is small, and if the contents exceed the above ranges, the spinnability of the fibres becomes inferior thereby to make their production difficult and degrade their quality.

The fire retardant used in the present invention may be suitably selected from known materials. Of these, organic halogen compounds are preferable, and concretely preferable examples thereof are decabromodiphenyl oxide (decomposition temperature: 350°C; the temperatures inside the following parentheses likewise indicating decomposition temperature), perchloropentacyclododecane (650°C), ethylenediamine dihydrobromide (355°C), hexabromobenzene (340°C), 2,2-bis[4-(2,3-dibromopropoxy)-3,5-dibromophenyl]propane (270°C), tris(2,3-dibromopropyl)phosphate (260°C), bis[3,5-dibrom-4-dibromopropyloxyphenyl]sulfone (280°C), etc.

These fire retardants are also preferably used in admixture with Sb₂0₃ in a ratio of retardant to Sb₂0₃ in a ratio of 1.5:1 to 3:1.

The fire retardants used in the present invention have a particle size of 62 pm or less. If the fire retardants contain particles larger than 62 microns, this causes reduction in their productivity or quality, , due to, e.g., clogging of spinning nozzle, fibre breakage at the time of stretching, forming of rough surface on fibres which lowers their heat adhesive properties.

The fire retardants having a particle size of 62 pm or less may be obtained by grading commercially available fire retardants by way of a known method such as a precipitation method, cyclone method, etc., and as a simpler method, by grading them through sieves indicated in JIS Z8801 (nominal diameter 62 or 53 11m).

The fire retardant composite fibres of the present invention may be produced according to a conventional melt-composite-spinning process and the apparatus employed may also be a conventional apparatus. As an example, a powdery raw material polymer having a fire retardant mixed is melted and extruded by a melt-extruder and the resulting melt is passed through a temperature-controlled heating zone to heat it to a definite temperature (hereinafter often referred to as spinning temperature). The melting and temperature adjustment of the polymer are carried out in separate passages for each of the composite components, and the respective composite components each having a definite temperature are fed in a composite ratio into spinning nozzles through the holes of which they are composite-spun. In the present invention, for the respective composite components, there is used a fire retardant having a decomposition temperature higher than the melting point of the components by 100°C or more, preferably higher than the spinning temperatures by 40°C or more, thereby to prevent the decomposition and consumption of the fire retardant at the time of spinning. Unstretched filaments obtained by the composite spinning are stretched in an appropriately chosen ratio depending on application fields. Usually the stretching is carried out very often in a stretch ratio of 4 or more. As the stretching temperature, temperatures in the range of from the softening point of the lower melting component up to a temperature lower than the melting point by 10°C may be employed, but the effect of the extent of the stretching temperature upon the fire retardant properties is little.

According to the process of the present invention, it is possible to produce composite fibers containing a large amount of a fire retardant and having a small fineness, with small frequencies of fiber breakage due to clogging of spinning nozzles and exchange of spinning die, in a stabilized manner and over an extremely long term. Further, the fire retardant composite fibers of the present invention are not only provided with fire retardant properties, but also, in spite of a large amount of fire retardant contained therein, have a smooth surface and superior heat adhesive properties.

The present invention will be further described by way of Examples and Comparative Examples. The terms and testing methods employed in these examples are as follows:
Particle size of fire retardant: this refers to the nominal dimension of meshes of standard sieves (JIS Z8801) employed for the grading, and means the largest particle size of the fire retardant.

Spinnability: this is classified by the number of fiber breakages per hour.
o: once or less, A twice, x: three times or more.

Life of spinning nozzle: this is classified by the exchange interval of spinning nozzle.
o: 40 hours or longer, Δ: 20 to 39 hours, x: shorter than 20 hours.

Adhesive strength: relative value of the adhesive strength of a sample non-woven fabric to its blank (a non-woven fabric prepared in the same manner as in the case of the sample except that it does not contain any fire retardant).
o: more than 90%, Δ: 70-90%, x: less than 70%.

Rough surface: the number of filaments having a rough surface among 100 filaments as observed by a microscope.
o: 2 filaments or less, A: 3-9 filaments, x: 10 filaments or more.

Content of fire retardant: Sb₂0₃ is regarded as an additive other than fire retardants.

Combustion test (JIS method): method according to JIS L1091, AI (45° microburner).

Combustion test (match method):
A sheet of a non-woven fabric was cut into a test piece of 3 cm long and 20 cm wide in the fiber direction. The resulting piece is then fixed so as to make an angle of 30° against the vertical surface and contacted with a flame of a match piece at the lower end of the piece from therebelow; till the sample piece catches the flame, and during the match piece is burnt, the lower end of the sample piece is burnt and the flame rises and is driven upwards from the lower end; just after the test piece has caught the fire, the match piece is drawn off, and the flame-remaining time is measured. Thus a sheet having a time of 5 seconds or shorter was defined as having passed the test, and that having a longer time was defined as failure.

### Examples 1-3 and Comparative Examples 1-4

As a lower melting component, a polyethylene (PE) having a melt flow rate (MFR) of 20 (according to JIS K7210, condition 4) and a melting point of 130°C, and as a higher melting component, a polypropylene (PP) having a MFR of 4 (according to JIS K7210, condition 14) and a melting point of 160°C, were used. Afire retardant (decabromodiphenyl oxide) having passed through a definite sieve as indicated in the Table shown later, in definite amounts relative to the PE and PP, respectively, as indicated in the Table, and Sb₂0₃ in of the respective amounts of the fire retardant were added to the PE and PP, separately. Composite spinning was then carried out in a composite ratio of 1:1, at a spinning temperature on the PE side of 230°C and at that on the PP side of 300°C to obtain unstretched side-by-side composite filaments having percentages fiber-cross-sectional circumference of the PE component of 78 to 85%. These filaments were stretched to 4 times the original lengths and cut to obtain staple fibers of 18d/F (deniers per filament; 20 dtex/F)x64 mm, which were then carded to prepare a web of 250 g/m^{2.}

This web was subjected to heat treatment at 140°C for 5 minutes to obtain a sheet of non-woven fabric of 15 mm thick, partially adhered on the PE side. This sheet was allowed to cool in a desicator for 3-4 hours, followed by carrying out combustion test according to the above JIS method to measure flame-remaining time (seconds) and carbonized area (cm²). Further, the same sheet of non-woven fabric was subjected to the above-combustion test according to the match method. The results of blending of fire retardants, spinning test and combustion tests are shown in the Table.

When Examples 1 and 2 are compared with Comparative Examples 1 and 2, and Example 3 is compared with Comparative Examples 3 and 4, even if the contents of a fire retardant in the whole of the fibers are the same, if the fire retardant is contained only in an amount less than 3% inside one of the composite components, the fire retardant effectiveness is inferior, and this is remarkable particularly in the evaluation according to the match method. Further, if the fire retardant is contained in an amount exceeding 15% inside one of the composite components, the spinning nozzle life becomes shorter and also the frequency of fiber breakage increases; hence such amount is also undesirable.

### Examples 4 and 5 and Comparative Examples 5-7

As a lower melting component, an ethylene-vinyl acetate copolymer (EVA) having a melting point of 110°C, a content of vinyl acetate component of 5% and a MFR of 25 (according to JIS K7210, condition 2) was used, and as a higher melting component, a polypropylene (PP) having a MFR of 4 was used. A blend of perchloropentacyclododecane as a fire retardant to Sb₂0₃ in a ratio of 2:1 was added in a definite amount to the PP and a blend of bis(3,5-dibrom-4-dibromopropyloxyphenyl)sulfone to Sb₂0₃ in a ratio of 1.5:1 was added in a definite amount to the EVA, as indicated in the Table. Composite spinning was then carried out in a composite ratio of 1:1 at a temperature of the lower melting component of 200°C and at that of the higher melting component of 280°C to obtain unstretched filaments which were then stretched to 4 times the original length and cut to prepare staple fibers (6d/Fx64 mm; 6.6 dtex/Fx64 mm) of sheath and core type composite fibers having a percentage fiber-cross-sectional circumference of the lower melting component of 100%, from which a sheet of non-woven fabric was prepared, followed by subjecting it to a combustion test as in Examples 1 and 2 to evaluate its fire retardant properties. The results are shown in the Table.

When Examples 4 and 5 are compared with Comparative Examples 5 and 6, it can be seen that if the particle size of the fire retardant exceeds 62 µm, spinnability and fiber quality become inferior, and if the spinning temperature is equal to its decomposition temperature, spinnability and fiber quality also become inferior due to a generated gas. Further it can be seen from Comparative Example 7 that even if the contents of a fire retardant in the whole of the fibers are the same, if the content of a fire retardant contained in one of the composite components is less than 3%, the fire retardant effectiveness is reduced.

### Examples 6 and 7 and Comparative Examples 8-11

As a lower melting component, a polyethylene (MFR: 10) (PE) was used and as a higher melting component, a polypropylene (MFR: 8) (PP) was used. Blends of tris(2,3-dibromopropyl)phosphate, 1,2-dibrom-3-chloropropane or pentadibromomonochlorocyclohexane as a fire retardant, each in a definite amount, to Sb₂0₃ in an amount in a ratio of the fire retardant to Sb₂0₃ of 3:1 were respectively added in a definite amount to PE, while a blend of ethylenediamine dihydrobromide to Sb₂0₃ in a ratio of 2:1 was added in a definite amount to PP, as indicated in the Table. Composite spinning was then carried out at a temperature on the lower melting component side of 210°C and at that on the higher melting component side of 300°C, in a composite ratio of 1:1 to obtain unstretched filaments which were then stretched to 4 times the original length and cut to obtain staple fibers of side by side composite fibers (3d/Fx64 mm; 3.3 dtex/Fx64 mm) having a percentage fiber-cross-sectional circumference of the lower melting component of 49-50%. A sheet of non-woven fabric was prepared from the staple fibers as in Examples 1 and 2 to evaluate the fire retardant properties. The results are shown in the Table.

As apparent from these results, in the case where the fineness of fibers is small, the particle size of fire retardant has a great influence upon spinnability (see Comparative Example 8 and 9); if a fire retardant is contained in the respective composite components in an amount of 12% (less than 15%) (the content of the fire retardant in the whole of the fibers being 12%), the spinnability and fiber quality are both inferior (see Comparative Example 11); and if a fire retardant having a decomposition temperature equal to spinning temperature is used, spinning is impossible at all (see Comparative Example 10).

## Claims

1. Fire retardant composite fibres comprising a fibre-formable polyolefin polymer as a higher melting component and as a lower melting component a polyolefin polymer having a melting point lower than that of the higher melting component by 10°C or more, there being a fire retardant in the respective components,
which composite fibres are characterized in that a fire retardant having a decomposition temperature higher than the melting point of the respective components by 100°C or more and also having a particle size of 62 pm or less, is present in the respective component in an amount of 3 to 15% by weight, the total amount of the fire retardant in the composite fibres being 5 to 10% by weight.

2. Fire retardant composite fibres according to claim 1, wherein the higher melting component is polypropylene or a copolymer composed mainly of propylene and the lower melting component is polyethylene or a copolymer composed mainly of ethylene, and the or each fire retardant added to these components has a decomposition temperature of 270°C or higher.

3. A process for producing fire retardant composite fibres by using a fibre-formable polyolefin polymer as a higher melting component and as a lower melting component a polyolefin polymer having a melting point lower than that of the higher melting component by 10°C or more, blending a fire retardant with the respective components and subjecting the resulting components to melt-composite-spinning followed by stretching,
which process is characterized by blending with the respective component a fire retardant having a decomposition temperature higher than the melting point of the respective components by 100°C or more and also having a particle size of 62 um or less, so as to give an amount of the fire retardant of 3 to 15% by weight, and also so that the total amount of the fire retardant in the composite fibres is 5 to 10% by weight; melting the resulting components at a temperature lower than the respective decomposition temperatures of the fire retardant contained in the respective components to subject them to composite spinning.

4. A process for producing fire retardant composite fibres according to claim 3, wherein fire retardants added to the higher melting component and the lower melting component are organic halogen fire retardants having a decomposition temperature higher than the respective spinning temperatures of the composite components by 40°C or more.

## Patentansprüche

1. Feuerhemmende Verbundfasern mit einem faserbildenden Polyolefinpolymer als einer höherschmelzenden Komponente und mit einem Polyolefinpolymer, dessen Schmelzpunkt um 10°C oder mehr unter dem der höherschmelzenden Komponente liegt, als einer niedrigschmelzenden Komponente sowie mit einem feuerhemmenden Mittel in den genannten Komponenten, wobei die Verbundfasern dadurch gekennzeichnet sind, daß ein feuerhemmendes Mittel mit einer Zersetzungstemperatur, die um 100°C oder mehr höher ist als der Schmelzpunkt der jeweiligen Komponenten, und mit einer Teilchengröße von 62 um oder weniger in den jeweiligen Komponenten in einer Menge von 3 bis 15 Gew.-% enthalten ist, wobei die Gesamtmenge des feuerhemmenden Mittels in den Verbundfasern 5 bis 10 Gew.-% beträgt.

2. Feuerhemmende Verbundfasern nach Anspruch 1, dadurch gekennzeichnet, daß die höherschmelzende Komponente Polypropylen oder ein hauptsächlich aus Propylen zusammengesetztes Copolymer und die niedrigschmelzende Komponente Polyäthylen oder ein hauptsächlich aus Äthylen zusammengesetztes Copolymer ist und daß das feuerhemmende Mittel oder jedes der diesen Komponenten zugesetzten feuerhemmenden Mittel eine Zersetzungstemperatur von 270°C oder darüber besitzt.

3. Verfahren zur Herstellung feuerhemmender Verbundfasern unter Verwendung eines faserbildenden Polyolefinpolymers als einer höherschmelzenden Komponente und eines Polyolefinpolymers mit einem Schmelzpunkt, der um 10°C oder mehr unter dem der höherschmelzenden Komponente liegt, als einer niedrigschmelzenden Komponente, durch Vermischen eines feuerhemmenden Mittels mit den jeweiligen Komponenten, wobei die entstehenden Komponenten dem Schmelz-Verbund-Spinnverfahren unterworfen werden, und anschließend gereckt wird, dadurch gekennzeichnet, daß mit den jeweiligen Komponenten ein feuerhemmendes Mittel vermischt wird, das eine Zersetzungstemperatur aufweist, die um 100°C oder mehr höher ist als der Schmelzpunkt der jeweiligen Komponenten und außerdem eine Teilchengröße von 62 um oder weniger besitzt, und zwar in einer Menge von 3 bis 15 Gew.-% an feuerhemmendem Mittel, derart, daß die Gesamtmenge des feuerhemmenden Mittels in den Verbundfasern 5 bis 10 Gew.-% beträgt, sowie dadurch, daß die entstehenden Komponenten bei einer Temperatur geschmolzen werden, die unter der der jeweiligen Zersetzungstemperaturen des feuerhemmenden Mittels, das in den jeweiligen Komponenten enthalten ist, liegt, und zu einem Verbund versponnen werden.

4. Verfahren nach Anspruch 3 zur Herstellung feuerhemmender Verbundfasern, dadurch gekennzeichnet, daß die feuerhemmenden Mittel, die der höherschmelzenden Komponente und der niedrigschmelzenden Komponente zugegeben werden, organische, Halogen enthaltende feuerhemmende Mittel mit einer Zersetzungstemperatur sind, die um 40°C oder mehr höher ist als die jeweiligen Spinntemperaturen der Verbundkomponenten.

## Revendications

1. Fibres composites retardatrices de flamme comprenant un polymère polyoléfinique formable en fibres comme composant à point de fusion supérieur et comme composant à point de fusion inférieur un polymère polyoléfinique ayant un point de fusion inférieur de 10°C ou plus au point de fusion supérieur, chaque composant comportant un retardateur de flamme, les fibres composites étant caractérisées en ce qu'un retardateur de flamme ayant une température de décomposition supérieure aux points de fusion des composants respectifs de 100°C ou plus et ayant aussi une taille de particules de 62 micromètres ou moins, est présent dans le composant respectif en une quantité égale à 3 à 15% en poids, la quantité totale de retardateur de flamme dans les fibres composites étant de 5 à 10% en poids.

2. Fibres composites retardatrices de flamme selon la revendication 1, dans laquelle le composant à point de fusion supérieur est le polypropylène ou un copolymère composé principalement de propylène et le composant à point de fusion inférieur est le polyéthylène ou un copolymère composé principalement d'éthylène, et le ou chaque retardateur de flamme ajouté à ces composants a une température de décomposition de 270°C ou plus.

3. Procédé de fabrication de fibres composites retardatrices de flamme utilisant comme composant à point de fusion supérieur un polymère polyoléfinique formable en fibres et comme composant à point de fusion inférieur un polymère polyoléfinique ayant un point de fusion inférieur de 10°C ou plus à celui du composant à point de fusion supérieur mélangeant un retardateur de flamme aux composants respectifs et soumettant les composés résultants à une opération de filage de composite à l'état fondu puis à un étirage caractérisé par le mélange avec chaque composant respectif d'un retardateur de flamme ayant une température de décomposition supérieure de 100°C ou plus aux points de fusion des composants respectifs et ayant aussi une taille de particules de 62 micromètres ou moins, de manière à obtenir une quantité de retardateur de flamme de 3 à 15% en poids et de manière aussi que la quantité totale de retardateur de flamme est de 5 à 10% en poids; la fusion des composants résultants à une température inférieure aux températures de décomposition respectives des retardateurs de flamme contenus dans les composants respectifs pour les soumettre à une opération de filage de composite.

4. Procédé de fabrication de fibres composites retardatrices de flamme selon la revendication 3 dans lequel les retardateurs de flamme ajoutés au composant à point de fusion supérieur et au composant à point de fusion inférieur sont des composés halogénés organiques retardateurs de flamme ayant une température de décomposition supérieure de 40°C ou plus aux températures respectives de filage des composants composites.
